

## UNITED STATES PATENT OFFICE.

ADOLF WELTER, OF DREIRINGWERKE, GERMANY.

## PROCESS FOR PRODUCING SOAP.

No Drawing. Application filed June 28, 1926, Serial No. 119,225, and in Germany July 3, 1925.

This invention relates to processes for producing soap and more particularly durable soaps made by the milling process that do not change through influences of the air or 5 weather.

Efforts have long been made to produce soaps that will keep indefinitely, that do not become unsightly when stored for long periods, whose weight does not change appreciably and which retain their original shape even in the tropics. The only soaps that will 10 meet these requirements are the soaps made by the milling process; they are formed or cut into strips by being passed through pairs of rolls and then pressed into cakes. These soaps will keep for practically any length of time because they have a high content of fatty acid and a low content of water. The only known method of producing them, apart 15 from the compressing of pure, non-hydrous, powdered soap, has consisted hitherto in milling. In the milling process liquid high grade grain soap is first solidified, and then cut into slices or rolled into bands so as to 20 make it present as large a surface as possible in the ensuing drying process. Although this drying process has recently been greatly improved by the use of ingeniously designed devices it still requires an amount of heat, 25 time and labor that is high in proportion to the value of the soap obtained. After the content of water has been reduced by this known method to such an extent that the content of fatty acid is about 80% the hard 30 soap is capable of being milled. The highest content of water at which the milling is possible at all is about 14 to 15% (see Schrauth, Medikamentöse Seifen 1914, page 30).

In practice it is, however, not advisable to 35 have the content of water above 10%. As to the content of fatty acid this must not be lower than 75% and the most favorable content for milling is 79-80%. Now I have found that, if the water in a hydrous soap 40 is partly or completely substituted by bicarbonate of sodium, it is possible to make easily millable and durable soaps even if the content of fatty acid is as low as 60 to 75%. The only process known up to the present by 45 which such soaps containing bicarbonate of sodium can be made cheaply consists in allowing fatty acids that are free of neutral fat to react directly on soda. When this is 50 done and one molecule of fatty acid and at

most one molecule of soda is used the following equation will hold:



Now it has been found that, if fatty acids 60 free of neutral fat as described are made to react on a maximum of one molecule of soda at about the melting temperature of the fatty acids and liquid or solid grain soap or even soap paste is added before, or even after, the 65 saponification is quite complete, a soap mixture is obtained which can be easily and perfectly milled and which has all the desirable properties such as durability, uniformity of composition, immutability of weight and 70 shape. Quite contrary to expectation this millability of the soap mixture was found to exist even when its content of fatty acid dropped to 60%, and even then rigorous conditions could be maintained in the method of 75 operation and imposed on the quality of the final product. It is, therefore, possible to produce high grade or grain soaps in this manner whose composition corresponds to that of ordinary grain soap but which greatly surpass it in respect to external appearance and 80 durability. My novel process has, however, further advantages which will now be gone into.

It is well known that in milling grain soap 85 the palm kernel or cocoanut oil content can only be up to 15%; if 20% is exceeded trouble ensues when milling. My aforescribed process, however, makes it possible not only to greatly increase the content of cocoanut or 90 palm kernel oil, but it even renders it possible to use this oil alone, which is extremely important as far as the solubility, foam forming qualities and the utility of the soap in sea- 95 water is concerned.

It is to be particularly noted that the aforescribed process supercedes by far all hitherto known processes in regard to economy and simplicity and that it enables a large production to be achieved even with a small plant. 100 Just as important is the fact that it enables marketable, nice-looking soap to be made from the prepared fatty acids in one to two hours, whereas the time required with known processes even with a perfect plant was several days. My novel process also enables a part of the soda to be replaced by crystallized sodium carbonate (washing soda) or by 105

potash and permits of the use of resin. Furthermore fat solvents such as hydrocarbon bodies, for example naphtha, kerosene, or benzol, hydro-naphthaline, hydro-phenol, 5 carbon-tetrachloride or the like may be used in the first stage of saponification or mixed with grain soap or soap paste to obtain milled soaps with a content of fat solvents.

10 *Example 1.*

1000 kgs. of palm kernel oil fatty acid or cocoanut oil fatty acid, containing more than 99% of free fatty acid, are mixed with 360 kgs. of water-free sodium carbonate. This 15 gives a uniform substance which saponifies after a while by spontaneous heating. Before the process of saponification is ended and before the substance has completely solidified, 700 to 800 kgs. of liquid grain soap, made 20 from tallow or bone fat, is added. By stirring or mixing these ingredients an almost homogeneous soap is obtained in a short time which after one hour can be milled in a milling machine into ribbons. These ribbons can be 25 formed immediately, or after they have been stored for a short period, into bars by a plodder or compressor and then cut into cakes or tablets.

30 *Example 2.*

30 1000 kgs. of a mixture consisting of 30% palm kernel oil fatty acid, 30% palm oil fatty acid, 40% tallow fatty acid, all split about 99% is stirred up with 350 kgs. of water-free 35 sodium carbonate at 30 to 35° C. At first this

substance is a thin liquid and perfectly homogeneous. After a short while it becomes warm and hardens, its temperature rising to 60 to 65° C. The saponification is complete in a few hours and the substance is then soluble in distilled water at a temperaure of 40 to 50° C. The solid substance is ground in a suitable mill as fine as possible and then mixed with liquid or solid grain soap. 400 kgs. of liquid grain soap is put into a mixing machine 45 and 600 kgs. of the aforesaid ground high grade soap substance is gradually added. After about 5, and at most 10, minutes a perfectly homogeneous substance is obtained which is converted by a single passage 50 through a mill into ribbons which are perfectly uniform and whose exterior does not differ in the least from the usual fine soap ribbons. These ribbons can be easily plodded, cut, and pressed, and their durability is in no 55 wise inferior to that of the finest soaps.

I claim:—

A process for producing air-resisting moulded soap consisting in mixing commercial fatty acids at about their melting 60 point with a quantity of alkali carbonate free from water, sufficient to saponify up to twice the quantity of fatty acids present, and after saponification, admixing grain soap therewith and thereupon subjecting the product 65 thus obtained to the milling process.

In testimony whereof I have affixed my signature.

ADOLF WELTER.